

Nov. 22, 1932.

W. BARR ET AL

1,888,755

DETERMINING THE SAFE WORKING STRESS OF METALS AT ELEVATED TEMPERATURES

Filed Oct. 3, 1931

2 Sheets-Sheet 1



William Barr & William Edward Barratt inventors  
per *A. D. Tracy, patent agent* ATTORNEY.

Nov. 22, 1932.

W. BARR ET AL

1,888,755

DETERMINING THE SAFE WORKING STRESS OF METALS AT ELEVATED TEMPERATURES

Filed Oct. 3, 1931

2 Sheets-Sheet 2

Fig. 2.

| TEMPERATURE<br>IN<br>°C | INITIAL<br>STRESS       | DECREASE                |
|-------------------------|-------------------------|-------------------------|
|                         | IN<br>TONS PER SQ. INCH | IN<br>TONS PER SQ. INCH |
| 400                     | 4.70                    | .30                     |
| 400                     | 6.70                    | 1.00                    |
| 400                     | 8.00                    | 1.35                    |
| 450                     | 3.00                    | .35                     |
| 450                     | 5.00                    | 1.52                    |
| 450                     | 7.00                    | 2.46                    |
| 500                     | 1.50                    | .36                     |
| 500                     | 3.00                    | 1.52                    |
| 500                     | 4.50                    | 2.55                    |
| 550                     | 1.00                    | .46                     |
| 550                     | 2.00                    | 1.36                    |

Fig. 3.



William Barr & William Edward Bardett INVENTOR.  
per N. D. Chapman ATTORNEY

## UNITED STATES PATENT OFFICE

WILLIAM BARR, OF HAMILTON, AND WILLIAM EDWARD BARDGETT, OF GLASGOW,  
SCOTLAND, ASSIGNEES TO COLVILLES LIMITED, OF GLASGOW, SCOTLAND

## DETERMINING THE SAFE WORKING STRESS OF METALS AT ELEVATED TEMPERATURES

Application filed October 3, 1931. Serial No. 566,754.

This invention relates to an improved means of and apparatus for determining the safe working stress of metals such as iron and steel and also non-ferrous metals and 5 their alloys which are subjected to stress at elevated temperatures; it being highly desirable to know the maximum stress which a metal can withstand indefinitely at a given temperature without undergoing any pronounced "creep", or plastic extension, due to 10 the combined effects of stress and temperature.

An object of the invention is to make provision whereby the safe working stress of 15 metals at elevated temperature can be determined with sufficient accuracy to meet all practical requirements and also within the space of a comparatively short time.

By careful experiments, we have ascertained that, under the continued action of 20 heat at constant temperature and of gradually decreasing stress, a piece of metal extends plastically due to creep at a progressively decreasing rate. We have also ascertained that the average rate of creep, during 25 a period of time commencing when the initial stress is applied, is proportional to the initial stress. So that, a decreased initial stress gives a decreased rate of creep; or, in other 30 words, the lower the initial stress the less will be the creep at the end of a given time. Thus, it follows that there will be a certain initial stress which will give no measurable creep during the said period and which therefore 35 will be a safe working stress.

Applying the knowledge derived from our experiments to the attainment of the objects of the present invention, specimens of a metal to be tested are heated to a selected temperature and subjected to different initial stresses, and, for a selected period, the temperature is maintained constant while the stresses gradually decrease as the metal elongates or creeps, the rates of decrease being proportionate to the creep experienced by the respective specimens. At the end of the said period, the decreases in stress experienced by the respective specimens are evaluated, and the safe working stress is determined mathematically, preferably graphically, from the

relationships between the initial stresses and the corresponding decreases in stress.

In order to control the decrease in stress, and at the same time to measure the stress, we preferably make use of "weigh bars" to 55 which we operatively connect the respective specimens. By the term "weigh bar" is meant a calibrated elastic body the physical properties of which are known and which accordingly serves as a measure of the stress 60 to which the specimen operatively connected to it is being subjected.

In order that the method and apparatus whereby our objects are attained can be clearly understood, reference will now be made by 65 way of example to the accompanying drawings, in which:—

Fig. 1 is a sectional elevation showing diagrammatically apparatus for use in determining the safe working stress of metals according to this invention.

Fig. 2 is a table of values obtained in a series of tests performed at different temperatures by the use of the said apparatus.

Fig. 3 is a view showing how the safe 75 working stresses at the respective temperatures are graphically determined from the said values.

Referring first to Fig. 1, the apparatus 80 therein shown comprises a battery of three units, and since these units are identical only one of them will be particularly described.

As shown, each unit includes a rigid rectangular frame 1 formed at the top and bottom with openings 1<sup>a</sup> and 1<sup>b</sup>. A bar 2 passing through the top opening of the frame 1 has a square-section portion 2<sup>a</sup> which fits 85 neatly through a square hole in a ring plate 3 secured to the top of the frame. The bar 2 is thus permitted to slide endwise through the plate but is constrained against turning movement. The upper part of the bar 2 is screw-threaded, being in engagement with a nut 4 on top of the plate 3, and a thrust-bearing 4<sup>a</sup>, for example a ball-bearing, may 90 be interposed between the plate 3 and nut 4. A bar 22 is suspended from below the bar 2 by a universal joint 23. A round bar 5 is adapted to be passed through the lower opening of 95 the frame 1, to the bottom of which a plate 100

6 is secured in way of said opening. The plate 6, which constitutes an anchorage for the bar 5, has a cup-shaped bearing adapted to accommodate a partly spherical facing 5<sup>a</sup> on the bottom end of the bar 5. There is also provided an intermediate connecting bar 7.

The unit includes an electric furnace 8 which can be set up within the frame 1 upon a platform 9 supported by flexible suspension cables 10 passing over the top of the frame.

The letters S and W respectively indicate the specimen to be tested and a calibrated steel bar constituting a weigh bar.

There is also provided a delicate extensometer of any appropriate form, for example as indicated by 11.

Before describing a test as performed by use of the battery of units, we shall describe what takes place in a single unit preparatory to and during the test.

The parts 2, 5, 7, S and W are assembled as shown in the drawings, the specimen S being secured to the bars 22 and 7, the weigh bar W being connected between the bars 5 and 7, and the extensometer being fitted to the weigh bar. In order that the parts W and S can be firmly secured, they may for example be provided with screw-threaded extensions (whose outlines are shown in dotted lines) adapted to be screwed into screw-threaded holes in the adjoining ends of the parts 2, 5 and 7.

The electric furnace 8 is energized and the current regulated to, and kept at, that value which maintains the specimen S at a selected temperature, the current being thermostatically controlled in known manner.

The nut 4 is turned so as to place the specimen and weigh bar under a predetermined initial stress, the magnitude of which would be greater than the roughly anticipated magnitude of the safe working stress at a selected temperature. The magnitude of the initial stress imposed by turning the nut 4 is directly obtainable from the reading indicated by the extensometer 11, as said magnitude is a known function of the elastic strain or extension imparted to the weigh bar W.

As the test proceeds the specimen S gradually elongates, or "creeps", due to the combined influences of stress and temperature. As the specimen creeps, the stress to which the weigh bar W is subjected becomes proportionately decreased, and consequently the specimen S is automatically subjected to a gradually decreasing stress, the magnitude of the decrease being continuously obtainable from the extensometer reading.

In carrying out the actual test, three similar specimens of a metal whose safe working stress is required are taken and are fitted into the respective units. The temperature of the three electric furnaces 8 is so regulated that the three specimens are all maintained at

precisely the same predetermined temperature throughout the test. At the commencement of the test, the three specimens are subjected to materially different initial stresses whose values are noted. The test may endure 70 for a period of time which may be about two days. We recommend this period, firstly, because of the need for a comparatively short test and, secondly, because a large proportion of the creep takes place in the first forty- 75 eight hours.

At the end of the test period, the extensometers are read and the values of the respective decreases in stress are noted. These values, together with those of the corresponding initial stresses, suffice to enable one to determine the safe working stress of the metal under test, at the respective temperatures, as will now be explained.

As previously stated, the lower the initial stress, the less will be the rate of creep, and accordingly the decrease of stress at the end of the test will also be less. We have ascertained that the mathematical law governing the relationship between the initial stresses and the corresponding decreases in stress can be graphically represented by a straight line. Thus it will be clear that two or more values of both initial stress and decrease in stress over a given period enable one to calculate, or estimate graphically, that initial stress which will give no measurable decrease in stress, the said initial stress being as aforesaid the safe working stress of the metal under test.

In order that the above statements can be clearly understood, we shall describe an actual series of tests with reference to Figs. 2 and 3.

The metal under test was mild steel containing .11% carbon, .01% silicon, .018% sulphur, .008% phosphorus and .56% manganese. A series of tests as above described was carried out at temperatures of 400° C., 450° C. and 500° C. and one further test was carried out with the use of only two units of the battery at 550° C. The values in tons per square inch of the initial stresses and decreases in stress are tabulated in Fig. 2. Graphs for the series of tests are shown in Fig. 3, the values of the decreases in stress being the ordinates and the values of the initial stresses being the abscissæ. It will be clear that the point where each of the respective graphs meets the base line denotes the maximum initial stress which will give no measurable decrease in stress at the temperature concerned, and also that this maximum initial stress will be the safe working stress. It will be seen from Fig. 3 that the values in tons per square inch of the safe working stress for the series are roughly 3.75, 2.3, 1 and .5, these values being arranged in the same order as the tests tabulated in Fig. 2.

It will be clear that a safe working stress can be obtained merely by performing tests 130

on two specimens. It will however be apparent that more accurate results can generally be obtained by having at least three units in the battery. It will also be apparent that 5 tests at one temperature need not be performed concurrently so long as the period of duration is the same, but where speed is an important factor all tests at one temperature should be carried out concurrently by use of 10 a battery of units.

We claim:—

1. A method of determining the safe working stress of metals at a selected temperature, which consists in subjecting specimens of a 15 metal while at said temperature to different initial stresses, allowing said stresses to decrease under the creep of the specimens themselves for a selected period of time, ascertaining the different creep values at the end 20 of said period, and evaluating the safe working stress of the metal at said temperature from the relationship between said values and the corresponding initial stresses.

2. A method of determining the safe working stress of metals at a selected temperature, which consists in taking separate specimens of a metal, heating these specimens to and maintaining them at said temperature, elastically subjecting the respective specimens to different initial stresses whereby they experience creep, allowing said stresses gradually to decrease under the automatic action of said creep for a selected 35 period of time, ascertaining the respective decreases in stress at the end of said period, and evaluating from said decreases and the corresponding initial stresses the safe working stress of the metal at said temperature.

3. A method of determining the safe 40 working stress of metals at a selected temperature, which consists in subjecting specimens of a metal while at said temperature to different initial stresses, allowing said stresses to decrease under the creep of the 45 specimens for a selected period of time, ascertaining the different creep values at the end of said period, ascertaining the decreases in stress corresponding respectively to said 50 creep values, and graphically determining the safe working stress of the metal at said temperature from the relationship between said decreases and the corresponding initial stresses.

4. A method of determining the safe 55 working stress of metals at a selected temperature, which consists in taking separate specimens of a metal, heating these specimens to and maintaining them at said temperature, elastically subjecting the respective 60 specimens to different initial stresses whereby they experience creep, allowing said stresses gradually to decrease under the automatic action of said creep for a selected 65 period of time, noting the different creep values at the end of said period, ascertaining

the decreases in stress corresponding respectively to said creep values, and graphically determining from said decreases and the corresponding initial stresses the safe working stress of the metal at said temperature.

5. A method of determining the safe working stress of metals at a selected temperature, which consists in concurrently subjecting specimens of a metal while at said temperature to different initial stresses, allowing 75 all said stresses to decrease concurrently under the creep of the specimens for a selected period of time, ascertaining the different creep values at the end of said period, and evaluating the safe working stress of the 80 metal at said temperature from the relationship between said values and the corresponding initial stresses.

6. A method of determining the safe working stress of metals at a selected temperature, 85 which consists in taking separate specimens of a metal, concurrently heating these specimens to and maintaining them at said temperature, elastically subjecting the respective specimens to different initial stresses whereby they concurrently experience creep, allowing said stresses gradually to decrease under the automatic action of said creep for a selected 90 period of time, ascertaining the respective decreases in stress at the end of said period, and evaluating from said decreases and the corresponding initial stresses the safe working stress of the metal at said temperature.

In testimony whereof we affix our signatures.

WILLIAM BARR.

WILLIAM EDWARD BARDGETT.

105

110

115

120

125

130